

## [54] ELECTROPHOTOGRAPHIC RECORDING MATERIAL WITH A PHOTOCONDUCTIVE CARBAZOLE COMPOUND

[75] Inventors: **Wilhelmus Janssens, Aarschot; Jozef Aime Dierckx, Mechelen; Hendrik Hubert, Wijnegem**, all of Belgium[73] Assignee: **Agfa-Gevaert, a naamloze vennootschap, Mortsel, Belgium**[22] Filed: **Sept. 21, 1973**[21] Appl. No.: **399,503**

## [30] Foreign Application Priority Data

Sept. 22, 1972 United Kingdom..... 44010/72

[52] U.S. Cl. .... **96/1.5; 96/1 R**[51] Int. Cl. <sup>2</sup> .... **G03G 5/04**

[58] Field of Search..... 96/1.5, 1 R

## [56] References Cited

## UNITED STATES PATENTS

|           |         |                     |        |
|-----------|---------|---------------------|--------|
| 3,341,472 | 9/1967  | Hewett.....         | 96/1.5 |
| 3,484,237 | 12/1969 | Shattuck et al..... | 96/1.5 |
| 3,642,480 | 2/1972  | Vrancken .....      | 96/1.5 |
| 3,652,269 | 3/1972  | Contois.....        | 96/1.5 |

Primary Examiner—Norman G. Torchin

Assistant Examiner—John L. Goodrow

Attorney, Agent, or Firm—William J. Daniel

## [57] ABSTRACT

Recording process comprising exposing to imagewise modulated electromagnetic radiation a photoconductive insulating recording element comprising an organic photoconductive compound corresponding to one of the following general formulae:

(I)



wherein:

each of Z<sub>1</sub> and Z<sub>2</sub> (the same or different) represents the necessary atoms to close an adjacent ring or ring system including such ring or ring system in substituted form,

Ar represents a bivalent aromatic group,  
each of R<sub>1</sub> and R<sub>2</sub> (the same or different) represents hydrogen, an aliphatic group including a cycloaliphatic group or said groups in substituted form, or an aryl group,

or R<sub>1</sub> and R<sub>2</sub> together represent the necessary atoms to close a nitrogen-containing ring including such a ring in substituted state.

(II)



wherein:

Z<sub>1</sub> and Z<sub>2</sub> have the same significance as described in general formula I,

A represents an alkylene group or an alkylene chain interrupted by a phenylene group, and

Ar represents a bivalent aromatic group.

8 Claims, No Drawings

**ELECTROPHOTOGRAPHIC RECORDING  
MATERIAL WITH A PHOTOCONDUCTIVE  
CARBAZOLE COMPOUND**

This invention relates to recording and reproduction of information-wise modulated electromagnetic radiation and to recording materials suitable therefor, and particularly relates to such processes and recording materials containing one or more organic photoconductive compounds as hereinafter described.

It has now been found that a particularly photosensitive photoconductive recording member can be formed by using in its composition a photosensitive compound corresponding to the following general formula:



wherein

each of  $Z_1$  and  $Z_2$  (the same or different) represents the necessary atoms to close an adjacent ring or ring system including such ring or ring system in substituted form, preferably an aromatic ring e.g. benzene ring in-

$Ar$  represents a bivalent aromatic group e.g. a phenylene group, and each of  $R_1$  and  $R_2$  (the same or different) represents hydrogen, an aliphatic group including a cycloaliphatic group or said groups in substituted form, e.g. an alkyl group including a substituted alkyl group e.g. methyl or benzyl, or an aryl group e.g. phenyl, or  $R_1$  and  $R_2$  together represent the necessary atoms to close a nitrogen containing ring including such ring in substituted state.

Preferred compounds according to the present invention that are particularly suited for use in electrographic recording materials are those wherein the atoms represented by  $Z_1$  and  $Z_2$  form a carbazole nucleus having on the nitrogen atom of the carbazole ring a phenyl group that is substituted in the p-position with the

20



group as defined.

The preparation of compounds used according to the present invention is illustrated by the following reaction scheme:



cluding a substituted aromatic ring e.g. a halogen-substituted benzene ring, the substituents being e.g. chlorine, bromine or iodine,

Suitable photoconductive compounds falling within the scope of the general formula are listed in the following table I.

Table I

| No. | Formula | melting point             |
|-----|---------|---------------------------|
| 1   |         | separated as oily product |

Table I -Continued

| No. | Formula                                                                             | melting point |
|-----|-------------------------------------------------------------------------------------|---------------|
| 2   |    | 184°C         |
| 3   |    | 129°C         |
| 4   |   | 212°C         |
| 5   |  | 231°C         |
| 6   |  | 122°C         |

## Preparation of compound 1 of table I

400 g of nitrobenzene were brought into reaction with 75 g of pulverized potassium hydroxide. The temperature of the reaction mixture was adjusted to 80°C with stirring. Then 100 g of carbazole were added portion wise in such a way that the temperature of the mixture continuously remained below 100°C.

After addition of the complete carbazole amount the mixture was kept for 30 min at 100°C. The whole was cooled overnight in a refrigerator. The residue was sucked off and washed with petroleum ether. The dried product was put into water and neutralized with acetic acid. The product obtained was sucked off and recrystallized from acetic acid or dichloroethane. A yellow

product corresponding to the following formula



was obtained. Melting point : 211°C. Yield : 50%.

A mixture of 39 g of N-(p-nitrobenzene)-carbazole and 3 ml of Raney nickel was brought to a volume of 240 ml with ethylene glycol monomethyl ether. Hydrogenation was performed at 1500 psi and 80°C. After 12 hours of shaking about 98% of the hydrogen had entered into reaction. The Raney nickel was filtered off, the solvent was evaporated and the residue was an oily product that slowly solidified.

#### Preparation of compound 2 of table I

A mixture of 0.02 mole of compound 1 of Table I, 0.05 mole of benzyl chloride, and 0.04 mole of pulverized anhydrous sodium carbonate in anhydrous ethanol was refluxed for 27 hours. The residue was sucked off, washed first with ethanol and afterwards with water to reach pH 7. Subsequently it was recrystallized from ethylene glycol monomethyl ether. A white product was obtained.

Melting point : 184°C.

Yield : 74%.

#### Preparation of compound 3 of Table I

A mixture of 0.02 mole of compound 1 of table I, 0.05 mole of benzyl chloride and 0.04 mole of pulverized anhydrous sodium carbonate was refluxed for 27 hours in anhydrous methanol. The residue was sucked off and consisted of compound 2. The mother lye standing for some days in a refrigerator yielded a second residue which upon recrystallization from ethyl alcohol yielded the compound 3 of Table I being a white product having a melting point of 129°C.

#### Preparation of compound 4 of table I

0.02 mole of compound 1 to table I was allowed to react with 0.066 mole of pulverized anhydrous potassium carbonate and 0.16 mole of trimethyl phosphate for 48 hours at 80°C. The whole was poured in a mixture of concentrated ammonium hydroxide and ice and stirred for 1 hour at ambient temperature. The product was sucked off, washed again with water to reach pH 7 and dried. Then it was crystallized from ethylene glycol monomethyl ether. A white product was obtained.

Melting point : 212°C.

Yield : 50%.

#### Preparation of compound 5 of table I

0.075 mole of compound 1 of table I was allowed to react for 16 hours on an oil-bath at 100°C with 0.05 mole of 1,2-dibromoethane and 0.1 g of triisopropanolamine. The residue was dissolved in 250 ml of chloroform and then boiled.

250 ml of 2N hydrochloric acid were added and the resulting mixture was shaken. A white product precipitated, which was filtrated.

Melting point : 200°-220°C.

By addition of 1N sodium hydroxide and after extraction with chloroform the hydrochloride was set free again. The extract was concentrated by evaporation of the volatile substances and thereafter it was boiled up with n-butanol.

The product was dissolved in hot dimethylformamide whereupon the same amount of methanol was added. Crystallization successively from dichloroethane and p-xylene with active carbon gave a white product melting at 231°C.

#### Preparation of compound 6 of Table I

A mixture of 0.1 mole of compound 1 of Table I, 0.05 mole of p-xylene dichloride and 0.1 mole of triisopropanolamine was heated gently on an oil-bath; the reaction went on suddenly at 90°C and the reaction mixture became solid. The temperature was increased to 125°C and afterwards the mixture was cooled. The pale hard mass was pulverized in a mortar with 2N hydrochloric acid, sucked off and washed with water until a neutral pH value was attained. Thereafter it was sucked off, washed with methanol and ether and recrystallized from ethylene glycol monomethyl ether. A white product was obtained.

Melting point : between 120° and 123°C.

Yield : 50 %.

The photoconductive compounds applied according to the present invention may be used alone or in combination with substances imparting desired chemical or physical properties to the recording element. So, these substances can be combined with other substances that either or not are photoconductive and exert an influence e.g. on the dark resistivity, the dischargeability or conductivity of the recording layer by an exposure to electromagnetic radiation, or on the transparency or the quality of the final image, e.g. by counteracting the fringe effect as described in the United Kingdom Patent Specification 1,007,349 filed December 12, 1961.

A proper combination with selected binding agents and/or chemical sensitizing agents may result in an enhancement of the total sensitivity. The recording elements according to the present invention preferably contain at least 5 % by weight of a photoconductive compound being within the scope of the above general formula. For use in electrophotography the recording element preferably consists for at least 10 % by weight of one or more of the said compounds. The electrically insulating binding agent used in a recording layer containing said photoconductive compound(s) may provide the desired mechanical strength e.g. to form a self-supporting layer, and preferably has a resistivity of at least 10<sup>9</sup> ohm. cm.

According to a particular embodiment the recording layer consists of the photoconductor, which, e.g., has been applied to a suitable support in molten state forming a micro-crystalline or glass-like layer on cooling. This technique can be applied when the photoconductive recording element has not to possess a high mechanical strength. For such technique reference is made to the Canadian Patent Specification 712,541 filed Feb. 5, 1960 by Gevaert Photo-Producten N.V.

Macromolecular compounds suitable for use as insulating binding agent for the photo-conductive compounds are, e.g., natural resins such as dammar resin, gum arabic, microcrystalline waxes, modified natural substances such as cellulose diacetate, cellulose triacetate, and ethylcellulose, pentaerythrite polyesters or modified colophony resins and ester gums, polymers such as polyethylene, polystyrene and copolymers of styrene, polyvinyl acetate and copolymers of vinyl acetate, polyvinyl acetals of formaldehyde, acetaldehyde or butyraldehyde, polyacrylic acid esters and polymethacrylic acid esters, coumarine-indene resins,

epoxy resins and polycondensates such as glycerol phthalate resins and other glyceryl polyesters, alkyd resins, diethylene glycol polyesters, formaldehyde resins and silicone resins.

Preferred binding agents are halogen-containing polymers. The sensitization of organic photoconductors with halogen-containing polymers is described in the United Kingdom Patent Specification 964,878 filed May 3, 1960 by Gevaert Photo-Producten N.V. According to said specification a material suitable for use in electrophotography comprises a photoconductive

5 layer incorporating an organic monomeric photoconductor and a halogen-containing polymer in such layer or in a juxtaposed layer (if any), the sensitivity of said photoconductor having been increased by making it to interact with said halogen containing polymer by heating.

In the following table II a list of preferred polymeric binding agents is given, which may be used in combination with the heterocyclic organic photoconductors of use according to the present invention as well as the corresponding suitable solvents.

Table II

| Polymeric binding agent defined by its structural unit(s)                                                                                                                                                     | Solvent            |
|---------------------------------------------------------------------------------------------------------------------------------------------------------------------------------------------------------------|--------------------|
| A repeating unit consisting of a central carbon atom bonded to a para-methoxyphenyl group (-O-C6H4-), a para-methoxyphenyl group (-C(CH3)(C6H4-O-)-), and two sulfonate groups (-SO2-).                       | methylene chloride |
| A repeating unit consisting of a central carbon atom bonded to a para-chlorophenyl group (-O-C6H4-), a para-chlorophenyl group (-C(CH3)(C6H4-Cl)-), and a decanoate group (-OOC-(CH2)8-CO-).                  | methylene chloride |
| A repeating unit consisting of a central carbon atom bonded to a para-methoxyphenyl group (-O-C6H4-), a para-methoxyphenyl group (-C(CH3)(C6H4-O-)-), and a carbonyl group (-O-C(=O)-).                       |                    |
| A repeating unit consisting of a central carbon atom bonded to a para-chlorophenyl group (-O-C6H4-), a para-chlorophenyl group (-C(CH3)(C6H4-Cl)-), and an oxygen atom (-O-).                                 | methylene chloride |
| A repeating unit consisting of a central carbon atom bonded to a hexamethylene group (-O-(CH2)6-O-), a decanoate group (-OOC-(CH2)8-CO-), and an oxygen atom (-O-).                                           | methylene chloride |
| A repeating unit consisting of a central carbon atom bonded to a para-methoxyphenyl group (-O-C6H4-), a para-methoxyphenyl group (-C(CH3)(C6H4-O-)-), and a dichloroacetyl group (-O-OC-CHCl-CHCl-CO-).       | methylene chloride |
| A repeating unit consisting of a central carbon atom bonded to a para-sulfonylphenyl group (-O2S-C6H4-SO2-), a para-sulfonylphenyl group (-O-C6H4-), and a para-methoxyphenyl group (-C(CH3)(C6H4-O-)-).      | methylene chloride |
| A repeating unit consisting of a central carbon atom bonded to a para-sulfonylphenyl group (-O2S-C6H4-C6H4-SO2-), a para-sulfonylphenyl group (-O-C6H4-), and a para-methoxyphenyl group (-C(CH3)(C6H4-O-)-). | methylene chloride |
| A repeating unit consisting of a central carbon atom bonded to a para-methoxyphenyl group (-O-C6H4-), a para-methoxyphenyl group (-C(CH3)(C6H4-O-)-), and a carbonyl group (-O-C(=O)-).                       | methylene chloride |

Table II -Continued

| Polymeric binding agent defined by its structural unit(s)                           | Solvent                                            |
|-------------------------------------------------------------------------------------|----------------------------------------------------|
|    | methylene chloride                                 |
|    | methylene chloride<br>25 % by weight               |
|    | methylene chloride                                 |
|   | methylene chloride                                 |
|  | methylene chloride                                 |
|  |                                                    |
|  | methylene chloride<br>10 % by weight               |
|  | 80 % by weight                                     |
|  | 10 % by weight                                     |
|  | 10 % by weight                                     |
|  | methylene chloride/acetone (1:1)<br>91 % by weight |
|  | 3 % by weight                                      |
|  | 6 % by weight                                      |
|  | methylene chloride/acetone (1:1)<br>85 % by weight |
|  | 14 % by weight                                     |
|  | 1 % by weight                                      |

Table II -Continued

Polymeric binding agent defined by its structural unit(s)



Solvent

methylene  
chloride/  
acetone/  
ethanol  
(1:1:1)

The photoconductive compounds applied according to the present invention can be used in admixture with other known inorganic and organic photoconductive substances, e.g. sulphur, selenium, photoconductive oxides, sulphides, and selenides of zinc, cadmium, mercury, antimony, bismuth, lead, anthracene, anthraquinone, and photoconductive polymers e.g. those containing N-vinylcarbazole recurring units and other known monomeric and polymeric organic photoconductors, e.g. those described in the published Dutch Patent Application 70/04174 filed Mar. 24, 1970 by Gevaert-Agfa N.V.

The inherent spectral sensitivity of most of the photoconductive compounds listed in Table I is mainly situated in the near U.V. range, i.e. in the range of 360 to 420 nm.

The spectral sensitivity of recording materials according to the present invention can be increased in different ways, e.g. by adding so-called spectral sensitizing agents for the photoconductive substances contained in the recording element or by admixing to the said heterocyclic organic photoconductive compounds other photoconductive substances, the inherent sensitivity of which for a particular part of the electromagnetic radiation spectrum is higher than that of the present compounds.

So, according to a special embodiment of the present invention semi-transparent recording layers are prepared, in which said photoconductive compounds are used in admixture with (an) inorganic photoconductive substance(s), especially photoconductive substances of the group of zinc oxide, photoconductive lead(II) oxide and photoconductive cadmium sulphide or cadmium selenide.

Suitable spectral sensitizing dyestuffs for the organic photoconductor are among others organic dyestuffs, known as methine dyes, or xanthene dyes of which the phthaleins and rhodamines are subclasses, and triarylmethane dyes e.g. crystal violet (C.I. 42,555) and the triarylmethane dyes described in published Dutch Patent Application 6704706 filed Apr. 3, 1967 by Gevaert-Agfa N.V. the term methine dyes includes mono- as well as polymethine dyes which dyes are known to those skilled in the art of the spectral sensitization of light-sensitive silver halide. Preferred methine dyes are of the cationic type. As preferred xanthene dyes Rhodamine B (C.I. 45,170), Rose Bengal (C.I. 45,440) and Fluorescein (C.I. 45,350) are mentioned. The spectral sensitizing dyes are preferably added to the recording layer composition in a proportion of 0.01 to 5% by weight in respect of the photoconductive substance(s).

Particularly preferred methine dyes are within the scope of the following general formulae:

I.



wherein:  
A<sub>1</sub> stands for a dimethine or tetramethine group including a substituted dimethine or tetramethine group,  
n stands for 1 or 2,  
R<sub>1</sub> stands for alkyl including substituted alkyl, an unsaturated aliphatic group e.g. allyl, aralkyl including substituted aralkyl, aryl including substituted aryl or cycloalkyl,  
R<sub>2</sub> stands for alkyl, aryl including substituted aryl, e.g. phenyl and phenyl substituted preferably in the p-position by alkyl, halogen and alkoxy, a 5- or 6-membered heterocycle the heteroatom of which is oxygen, sulphur, selenium or nitrogen such as 2-, 3-, or 4-pyridyl, 2-furyl, 2-thienyl, etc. including their quaternary salts,  
R<sub>3</sub> stands for hydrogen or has one of the meanings given for R<sub>1</sub>,  
R<sub>4</sub> stands for hydrogen, alkyl, alkoxy or halogen or together with R<sub>3</sub> forms an alkylene bridge such as dimethylene and trimethylene,  
each of R<sub>5</sub> and R<sub>6</sub> (the same or different) stands for hydrogen, alkyl, alkoxy or halogen or together represent the atoms necessary to complete a fused-on benzene nucleus,  
X<sub>1</sub><sup>-</sup> represents an anion e.g. Cl<sup>-</sup>, Br<sup>-</sup>, I<sup>-</sup>, ClO<sub>4</sub><sup>-</sup>, CH<sub>3</sub>SO<sub>4</sub><sup>-</sup>, or



but is missing when the R<sub>1</sub> group contains already an anion (betaine type salt), and Z represents the atoms necessary to complete a heterocyclic nucleus of the types used in the production of cyanine dyes e.g. such as those of the thiazole series e.g. thiazole, 4-methylthiazole, 4-methyl-5-carbethoxythiazole, 4-phenylthiazole, 5-methylthiazole, 5-phenylthiazole, 4-

(p-toly)-thiazole, 4-(p-bromophenyl)-thiazole, 4,5-dimethylthiazole, 4,5-diphenylthiazole, 4-(2-thienyl)-thiazole, 4-(m-nitrophenyl)-thiazole, those of the benzothiazole series, e.g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-bromobenzothiazole, 6-sulphobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, 4,5,6,7-tetrahydrobenzothiazole, 5,6-dimethoxybenzothiazole, 5,6-dioxymethylenebenzothiazole, 5-hydroxybenzothiazole, 6-hydroxybenzothiazole, 5,6-di-methylbenzothiazole, those of the naphthothiazole series e.g. naphtho[2,1-d]thiazole, naphtho[1,2-d]thiazole, 5-methoxynaphtho[1,2-d]thiazole, ethoxynaphtho[1,2-d]thiazole, methoxynaphtho[2,1-d]thiazole, 7-methoxynaphtho[2,1-d]thiazole, those of the thionaph-

1-isoquinoline, 3,4-dihydroisoquinoline, those of the 3-isoquinoline series e.g. 3-isoquinoline, those of the pyrimidine series, those of the quinoxaline series, those of the quinazoline series, those of the 1-phthalazine series, those of the 2-pyridine series, e.g. pyridine, 5-methylpyridine, 3-nitropyridine, those of the 3,3-dialkylindolenine series, e.g. 3,3-dimethylindolenine, 3,3,5-trimethylindolenine, 3,3,7-trimethylindolenine, etc., those of the benzimidazole series e.g. benzimidazole, 5,6-dichlorobenzimidazole, 5-chlorobenzimidazole, 5,6-dibromobenzimidazole, 5-chloro-6-benzimidazole, 5-phenylbenzimidazole, 5-fluorobenzimidazole, 5,6-difluorobenzimidazole, 5-cyanobenzimidazole, 5,6-dicyanobenzimidazole, 5-chloro-6-cyanobenzimidazole, 5-fluoro-6-cyanobenzimidazole, 5-acetylbenzimidazole, 5-chloro-6-fluorobenzimidazole, 5-carboxybenzimidazole, 7-carboxybenzimidazole, 5-carbethoxybenzimidazole, 7-carbethoxybenzimidazole, 5-sulphamylbenzimidazole, or 5-N-ethylsulphamylbenzimidazole, 5-ethylsulphonylbenzimidazole and 5-trifluoromethylsulphonylbenzimidazole;

## II.



theno [7,6-d]-thiazole series e.g. 7-methoxythionaphtheno [7,6-d]-thiazole, those of the thiadiazole series e.g. 4-phenylthiadiazole, those of the oxazole series e.g. 4-methyloxazole, 5-methyloxazole, 4-phenyloxazole, 4,5-diphenyloxazole, 4-ethyloxazole, 4,5-dimethyloxazole, 5-phenyloxazole, those of the benzoxazole series e.g. benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 6-methoxybenzoxazole, 5-hydroxybenzoxazole, 6-hydroxybenzoxazole, those of the naphthoxazole series, e.g. naphtho[2,1-d]oxazole, naphtho[1,2-d]oxazole, those of the selenazole series e.g. 4-methylselenazole, 4-phenylselenazole, those of the benzoselenazole series e.g. benzoselenazole, 5-chlorobenzoselenazole, 5-methoxybenzoselenazole, 5-methyl-6-methoxybenzoselenazole, 5,6-dioxymethylenebenzoselenazole, 5-hydroxybenzoselenazole, 4,5,6,7-tetrahydrobenzoselenazole, those of the naphthoselenazole series e.g. naphtho[2,1-d]-selenazole, naphtho[1,2-d]-selenazole, those of the thiiazoline series e.g. thiiazoline, 4-methylthiazoline, 4-hydroxymethyl-4-methylthiazoline, 4,6-bis-hydroxymethylthiazoline, those of the oxazoline series e.g. oxazoline, those of the selenazoline series e.g. selenazoline, those of the 2-quinoline series e.g. quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc., those of the 4-quinoline series e.g. quinoline, 6-methoxyquinoline, 7-methylquinoline, 8-methylquinoline, those of the 1-isoquinoline series e.g.

wherein

$A_2$  stands for a monomethine or trimethine group including a substituted monomethine or trimethine group, each of  $R'_2-R'_6$  and  $R''_2-R''_6$  (the same or different) has one of the meanings given for  $R_2-R_6$ ,  $X_2^-$  has the same significance as  $X_1^-$ ;

## III.



wherein:

each of  $R'_1$  and  $R''_1$  (the same or different) has one of the meanings given for  $R_1$ ,  $X_3^-$  has the same meaning as  $X_1^-$ ,  $A_3$  has the same meaning as  $A_2$ ;

each of  $m$  and  $p$  (the same or different) stands for 1 or 2, and

each of  $Z_1$  and  $Z_2$  (the same or different) stands for the atoms necessary to complete a heterocyclic nucleus of the thiiazole, benzothiazole, naphthothiazole, thionaphtheno[7,6-d]-thiazole, thiadiazole, oxazole, benzoxazole, naphthoxazole, selenazole, benzoselenazole, naphthoselenazole, 2-quinoline, 4-quinoline, pyrimidine, quinoxazoline, 2-pyridine, 3,3-dialkylindolenine or of the benzimidazole series;

representative examples of these heterocyclic nuclei can be found above in the definition of  $Z$  in formula I.

The dyestuffs corresponding to the above general formulae can be prepared according to the methods known by those skilled in the art of methine dye chemistry.

According to a further embodiment of the invention, the recording material contains one or more substances that increase the photoconductivity of the recording material in the inherent spectral sensitivity range of the said heterocyclic organic photoconductive compounds. As already has been said a binding agent can act as a sensitizing agent that enhances the total sensitivity of the recording element. In this respect compounds are to be mentioned which contain one or more electron-attracting atoms or groups e.g. those that are known as non-ionic Lewis acids, e.g. the Lewis acids that can form a "charge transfer complex" as described in U.S. Pat. No. 3,408,183 of Joseph Mammino issued Oct. 29, 1968. Good sensitizing results are obtained with organic carboxylic acid anhydride compounds and with quinones containing electron-attracting substituents e.g. halogen or cyano, such as in tetrachlorobenzoquinone, tetracyanobenzoquinone and in organic compounds containing



group, and with the compounds according to the structural formula of the Belgian Patent Specification 734,141 filed June 6, 1969 by Gevaert-Agfa N.V. and the chlorine- and/or cyano-containing polymers of Table II.

The photoconductive compounds may be used in admixture with diazonium salts that on exposure to electromagnetic radiation produce (a) radical(s) that irreversibly increase(s) the electro-conductivity of a recording layer. Such substances as well as details about their incorporation into a recording layer containing an organic photoconductive insulating substance are described in the United Kingdom Patent Specification 964,872 filed Apr. 22, 1959 by Gevaert Photo-Producten N.V. and the U.S. Pat. No. 3,113,022 of Paul Maria Cassiers, Jean Marie Nys, Jozef Frans Willems and Rene' Maurice Hart issued Dec. 3, 1963. A particularly suitable conductivity-increasing diazonium compound is p-nitrobenzenediazonium chloride. The diazonium compounds are preferably used in an amount of 0.01 % to 10 % by weight in respect of the present photoconductive heterocyclic organic compounds.

Other additives well known in the art of preparing photoconductive coatings for recording purposes may be used, e.g. matting agents, fluorescing compounds, phosphors, optical brightening agents, agents controlling the adhesive power of the recording layer, agents controlling the elasticity, the plasticity and the hardness of the recording layer, agents controlling the viscosity of the coating composition, antioxidants, gloss-improving agents, etc.

Transparent and semi-transparent recording materials containing the photoconductive heterocyclic organic compounds are described hereinbefore are especially suited for use in recording materials applied for the production and reproduction of microfilm images. Microfilm images can be copied in contact or enlarged optically on recording materials according to the present invention. According to the type of development, the transparencies obtained (contact copies and en-

largements) can serve as negative or positive intermediate prints for further printing, e.g. on diazotype materials.

The semitransparent recording materials according to the present invention preferably have an optical density not larger than 0.30 towards visible light or the copying light used in the printing apparatus wherein it is used as intermediate print.

10 The photoconductive heterocyclic organic compounds described hereinbefore are further especially suited for use in the production of pigment images wherein the latter may have the properties of a fluorescent compound or phosphor. As is generally known luminescent phosphors are used in screens of cathode-ray tubes and more particularly in television, X-ray, radar and oscilloscope screens.

15 In colour television screens phosphors of different colour have to be fixed on a screen in a particular pattern.

20 The described photoconductive compounds are used successfully in a process for the production of colour television screens as described in the French Patent Specification 1,336,499 filed Sept. 26, 1962 by Comp.-

25 Francaise Thomson-Houston. According to the process described in said specification a pattern of a phosphor on a screen support is produced by the steps of applying to said support a coating of an electroconductive material and to said coating a layer comprising a vaporizable or thermolysable photoconductive compound

30 optionally incorporated in a vaporisable or thermolysable binding agent. On said coating an electrostatic charge pattern corresponding with the pigment pattern to be produced is formed in an electrophotographic

35 way, and the electrostatic charge pattern is developed with non-volatile powder particles that have the desired phosphorescent or luminescent properties. Subsequently, the photoconductive layer containing the phosphor powder image is heated to remove the volatile substances of the photoconductive recording layer and to make the phosphor pattern adhere to the screen support.

40 In order to fix the powder image before applying the heating step it is preferably overcoated with a layer of a thermolysable binding agent.

45 According to said French Patent Specification photoconductors of the group of anthracene, anthraquinone and xanthene are used. The recording layer may further contain boric acid.

50 The photoconductors mentioned in the French Patent Specification are advantageously substituted partly or wholly by the photoconductive substances applied according to the present invention.

55 Suitable thermolysable binding agents belong to the class of the polyacrylic acid esters and polymethacrylic acid esters, e.g. polymethyl methacrylate, polyethyl methacrylate and polyethyl acrylate.

60 The thickness of the photoconductive layers of the present invention is not critical but is open to choice within a wide range according to requirements in each individual case. Good results are attained with photoconductive layers of a thickness between 1 and 30  $\mu$  preferably between 2 and 20  $\mu$ . Too thin layers do not have a sufficient insulation power in the absence of active electromagnetic radiation, whereas too thick layers require extensive exposure times.

In the manufacture of electrophotographic recording materials according to the present invention a relatively conductive support for the recording layer is used, e.g. an electroconductive sheet or plate, or an insulating sheet or plate covered with an electroconductive interlayer. BY electro-conductive plate or sheet is understood a plate or sheet whose electrical resistivity is smaller than that of the non-irradiated (dark-adapted) photoconductive layer i.e. in general smaller than  $10^9$  ohm.cm and preferably is at least 100 times as small as that of the recording layer. Supports whose resistivity is not higher than  $10^7$  ohm.cm are preferred. The recording layers themselves preferably have an electrical insulating power as high as possible without affecting too much the photosensitivity by means of too high an amount of insulating binding agent. In non-irradiated state (dark-adapted state) the recording layers preferably have a resistivity of at least  $10^9$  ohm. cm.

Suitable conductive plates are, e.g. plates of metals such as aluminium, zinc, copper, tin, iron, or lead.

Suitable electro-conductive interlayers for insulating supports are, e.g. vacuum-coated metal and conductive metal compound (metal oxide or metal salt) layers such as silver, tin, aluminum, and copper iodide conductive layers, transparent conductive polymer layers, e.g. applied from polymers containing quaternized nitrogen atoms, such as those described in the United Kingdom Patent Specification 950,960 filed Sept. 23, 1960 by Gevaert Photo-Producten N.V., or layers containing conductive particles, e.g. carbon black and metal particles dispersed in a binder. The binder used for said particles has a resistivity preferably lower than  $10^6$  ohm.cm. A suitable binder for that purpose is gelatin.

It is possible to produce transparent photoconductive recording materials by applying the photoconductive compounds together with a suitable binder (if necessary) from a clear solution to a conductive transparent base or a transparent insulating base coated with an electroconductive transparent interlayer.

As transparent bases resin sheets having an optical density of not more than 0.10 are preferred, e.g. a sheet made of polyethylene terephthalate or cellulose triacetate. The conductive interlayer preferably consists of a metal coating, e.g., a vacuum-coated aluminium layer having an optical density of not more than 0.30, or of a conductive transparent polymer layer composed, e.g. of an organic polyionic polymer, e.g. a polymer containing quaternized nitrogen atoms such as a quaternized polyethylene-imine.

In reproduction techniques wherein the prints are to be produced on an opaque background preferably a paper sheet is used as support for the recording layer.

Paper sheets that have an insufficient electrical conductivity are coated or impregnated with substances enhancing their conductivity, e.g. by means of a conductive overcoat such as a metal sheet laminated thereto.

As substances suited for enhancing the conductivity of a paper sheet and which can be applied in the paper mass are particularly mentioned hydroscopic compounds and antistatic agents as described, e.g. in the United Kingdom Patent Specification 964,877 filed May 2, 1960 by Gevaert Photo-Producten N.V., and antistatic agents of polyionic type, e.g. CALGON

CONDUCTIVE POLYMER 261 (trade mark of Calgon Corporation, Inc. Pittsburgh, Pa., U.S.A.) for a solution containing 39.1% by weight of active conductive solids, which contain a conductive polymer having recurring units of the following type:



Paper sheets are preferably impermeabilized to organic solvents, e.g. by means of a water-soluble colloid or by strongly hydrating the cellulose fibers such as in the case of glassine paper.

In order to prepare an electrophotographic material according to the present invention various techniques may be applied.

In practice, the photoconductive substances involved, either alone or together with other additives such as those described above, preferably are first dissolved or dispersed in a suitable organic solvent such as a chlorinated hydrocarbon, e.g. methylene chloride. The solution or dispersion thus obtained is spread uniformly on a surface of a suitable support, e.g. by centrifuging, spraying, brushing, or coating. Thereupon the layer formed is dried in such a way that a solid photoconductive layers is formed on the surface of the support.

Recording materials according to the present invention can be used in any of the different techniques known in recording with the aid of photoconductors. According to a preferred embodiment they are used in a technique based on the discharge of an electrostatically charged recording layer by exposure to light.

Photoconductive recording materials prepared according to the present invention can be used in exposure units equipped with incandescent lamps, so that they need not be exposed to light rays rich in ultraviolet such as those emitted by a high-pressure mercury vapour bulb.

The electrostatic charging of photoconductive recording elements according to the present invention can be effected according to any method known in electrophotography, e.g. by friction with a smooth material, with a material possessing a high electric resistance, e.g. a cylinder coated with polystyrene, by corona discharge, by contact charge, or by discharge of a capacitor.

Recording materials containing the said organic photoconductive substances can be used in a recording technique comprising a negative corona charging as well as in a recording technique comprising a positive corona charging.

For the production of an electrostatic image it is possible to effect the charging and exposure steps simultaneously and even to expose the recording layer image-wise before the charging since a conductivity image is formed that is not destroyed immediately, especially when diazonium salts are used in the recording element. It is preferred, however, to perform the charging before the image-wise exposure.

The electrostatic latent image can be converted into a visible image either on the electrophotographic material wherein the latent image was formed, or on a material to which the electrostatic latent image was transferred, e.g. by application of the method described in the Belgian Patent Specification 529,234 filed May 29, 1954 by Chester Floyd Carlson.

The conversion of the original or transferred latent image into a visible image can occur according to one of the techniques known in electrophotography, wherein use is made of a conductivity pattern (e.g. electrolysis) or the electrostatic attraction or repulsion of finely divided coloured substances, which, e.g. are present in a powder mixture, in an electrically insulating liquid (e.g. in the form of a suspension) or in a gas (e.g. in the form of an aerosol), or wherein electrostatic attraction is used for selectively wetting charged portions of the recording layer, as described in the United Kingdom Patent Specifications 1,020,505 filed Nov. 8, 1961 and 1,033,419 filed Nov. 26, 1962 both by Gevaert Photo-Production N.V.

When the sign of the charge of the developing powder or developing liquid is properly chosen, either a negative or a positive print can be obtained from any original. If both printing material and developing powder or developing liquid have the same sign of charge, the powder only adheres to the discharged areas so that a negative print is obtained. If the signs of the recording material and of the developing powder or developing liquid differ, a positive print is obtained.

If a coloured powder is used for making visible the latent image, the visible image obtained can, if necessary, be fixed according to one of the methods known in electrophotography, e.g. by heating, or it can be transferred to another support, e.g. according to the method described in the United Kingdom Patent Specification 658,699 filed Apr. 14, 1949 by Battelle Memorial Institute and fixed thereon.

The present heterocyclic organic photoconductive compounds can also be supplied in a thermoplastic recording process to form a ripple-image as described, e.g. in the United Kingdom Patent Specification 964,881 filed May 17, 1960 by Gevaert Photo-Producten N.V.

Evidently, the present invention is by no means limited to one or other particular embodiment of using the electrophotographic material containing the photoconductive compounds as described herein. The exposure technique, the charging method, the formation of the charge pattern, the transfer of such pattern if applied, the developing method, and the fixation or the transfer of the developing material pattern may be modified or adapted.

The composition of the recording materials used in these methods may be adapted to the requirements of the recording process used.

Electrophotographic materials according to the present invention can be employed in reproduction techniques, wherein different kinds of electromagnetic radiations are used, e.g. visible light, U.V.-radiation, X-rays and  $\gamma$ -rays.

The present invention is illustrated by the following examples.

The percentages and ratios are by weight unless otherwise indicated.

## EXAMPLE 1

An aluminium-laminated paper sheet was coated with the following composition:

|    |                                                                                             |        |
|----|---------------------------------------------------------------------------------------------|--------|
| 5  | 10% by weight solution in methylene chloride of an organic photoconductor listed in Table I | 50 ml  |
| 10 | copoly(vinyl chloride/vinyl acetate/maleic anhydride) (molar ratio 86.5/13.3/0.2)           | 5 g    |
|    | 1,2-dichloroethane                                                                          | 45 ml. |

The coating was carried out in such a ratio that the dried photoconductive layer contained 2 g of photoconductor per sq.m.

15 After a negative corona charging with a potential difference of -6000 V between the corona wires and the ground, the charged recording layer was contact-exposed for 30 sec. through a step wedge having 0.20 log exposure increments. In this exposure 5 Osram (trade name) L 20 fluorescent tubes, mainly emitting in the U.V. range and the shorter wavelengths of the visible spectrum were placed at a distance of 20 cm from the recording layer.

20 The latent wedge image obtained was electrophoretically developed by means of an electrophoretic developer prepared by diluting the concentrated developer composition described hereinafter in a volume ratio of 15/1000 by means of ISOPAR H (an isoparaffinic hydrocarbon mixture having a boiling range of 177°-188°C sold by Esso Belgium N.V., Antwerp, Belgium):

|    |                                                                        |        |
|----|------------------------------------------------------------------------|--------|
| 35 | carbon black (average particle size : 20 nm)                           | 30 g   |
|    | zinc monotridecyl phosphate as dispersing agent                        | 1.5 g  |
|    | ISOPAR H (trade name) resin solution prepared as described hereinafter | 750 ml |
|    |                                                                        | 150 g. |

45 The resin binder solution was prepared by heating 500 g of ALKYDAL L 67 (a trade name of Farbenfabriken Bayer A.G., Leverkusen, W. Germany for a linseed oil-modified (67 % by weight) alkyd resin) and 500 ml of white spirit containing 11 % by weight of aromatic compounds at 60°C till a clear solution was obtained, and subsequent cooling.

50 A black positive copy of the wedge original on a transparent base was obtained.

From the wedge prints obtained the relative speed values of the developed materials were calculated based on a comparison of the number of non-toned (discharged) steps present in the wedge prints obtained with materials containing a photoconductor of Table I with the number of non-toned steps produced in a material containing photoconductor number 2 of Table I to which is given arbitrarily the speed value 100.

| Number of compound of Table I | Relative Speed values |
|-------------------------------|-----------------------|
| 2                             | 100                   |
| 1                             | 400                   |
| 3                             | 100                   |
| 4                             | 250                   |
| 6                             | 400                   |

21

## EXAMPLE 2

An electrophotographic recording material was prepared by coating onto an aluminium-laminated paper a solution containing:

10% by weight solution in methylene chloride of an organic photoconductor listed in Table I  
 copoly(vinyl chloride/vinyl acetate/maleic anhydride) (molar ratio 86.5/13.3/0.2)  
 Rhodamine B (C.I. Basic Violet 10 C.I. 45,170)  
 1,2-dichloroethane

50 ml  
 5 g  
 0.025 g  
 45 ml.

The dried recording layer contained 2 g of photoconductor per sq.m.

The coated samples were negatively charged with a negative corona having a potential difference of -6000 V between the corona wires and the ground.

The charged recording layer was contact-exposed for 6 sec. through a step-wedge having 0.20 log exposure increments. In the exposure tungsten filament light was used.

The latent wedge images were electrophoretically developed as described in Example 1.

The relative speed values of the developed materials were compared with those of the electrophotographic material containing photoconductor number 6 of Table I which is given arbitrarily the speed value 100.

| Number of compound of Table I | Relative speed values |
|-------------------------------|-----------------------|
| 1                             | 4                     |
| 2                             | 40                    |
| 3                             | 40                    |
| 4                             | 400                   |
| 5                             | 4                     |
| 6                             | 100                   |

## EXAMPLE 3

To a polyethylene terephthalate support of 100  $\mu$  a conductive transparent coating was applied from an aqueous solution of gelatin and CALGON CONDUCTIVE POLYMER 261 (trade mark) in a weight ratio of 2:1. Coating was carried out in such a way that the dried coating contained 2 g of gelatin per sq.m. The electrical surface resistance of the coating was  $1 \times 10^6$  ohm per sq.cm measured at a relative humidity of 50 %.

An electrophotographic recording material was prepared by coating onto said conductive layer a solution consisting of

methylene chloride  
 1,2 dichloroethane  
  
 copoly(vinyl chloride/vinyl acetate/maleic anhydride) (molar ratio 86.5/13.3/0.2)  
 $N(CH_3)_2$

45 ml  
 45 ml  
 5 g  
 5 g

22

-Continued

Rhodamine B (C.I. Basic Violet 10; C.I. 45,170) 0.025 g.

5

The dried recording layer containing approximately 3 g of photoconductor per sq.m was charged with a negative corona and contact-exposed with 500 lux.sec with the same light source as in Example 2. The latent image was electrophoretically developed for 5 sec with the developer described in Example 1. A good copy of the original was obtained.

## EXAMPLE 4

15 To a polyethylene terephthalate support of 63  $\mu$  a conductive transparent coating was applied from

20 a 10% aqueous solution of polystyrene sulfonic acid sodium salt 40 ml  
 methanol 60 ml.

25 The coating was carried out in such a way that the dried material contained 1.75 g of polystyrene sulfonic acid sodium salt per sq.m. The electrical surface resistance was  $5 \times 10^6$  ohm/cm<sup>2</sup> measured at a relative humidity of 50 %.

An electrophotographic recording material was prepared by coating at a coverage of 3 g/m<sup>2</sup> onto said conductive layer a solution containing:

35 compound 6 of Table I 5 g  
 methylene chloride 45 g  
 1,2-dichloroethane 45 g  
 PARLON P-20 (marketed by the Hercules Powder Company, Inc., Wilmington, Del. USA)  
 chlorinated polypropylene 66.89% of chlorine 5 g.

40

After a negative corona charging with a potential difference of -6000 V the charged recording layer was contact-exposed for 2 sec through a positive transparency of a test chart with 8 Osram (trade name) L 20 45 fluorescent tubes at a distance of 20 cm from the recording layer.

50 After the exposure the latent image was developed for 5 sec with a triboelectrically charged positive toner on the base of three parts by weight of pitch, 4 parts by weight of colophony and 3 parts by weight of carbon black.

A contrasty transparent positive copy of the transparency was obtained.

55

## EXAMPLE 5

The effect on the speed of electrophotographic recording materials resulting from a few chemical sensitizers was examined.

60 Therefore the following photoconductive compositions were coated on an aluminium-laminated paper:

65 10% by weight solution in methylene chloride of the organic photoconductor nr. 2 of Table I 50 ml  
 copoly(vinyl chloride/vinyl acetate/maleic anhydride) (molar ratio 86.5/13.3/0.2) 5 g  
 a chemical sensitizer listed in Table III below 0.05 g.

Table III

| Test no. | Structural formula<br>chemical sensitizer | relative<br>speed value |
|----------|-------------------------------------------|-------------------------|
| 0        | none                                      | 100                     |
| 1        |                                           | 250                     |
| 2        |                                           | 400                     |
| 3        |                                           | 600                     |
| 4        |                                           | 400                     |

EXAMPLE 6

Electrophotographic recording materials were prepared by coating onto a conductive layer as described in Example 3 a composition containing:

10 compound 6 of Table I  
copol(vinyl chloride/vinyl acetate/maleic anhydride)(Molar ratio 86.5/13.3/0.2)  
methylene chloride  
1,2-dichloroethane  
a sensitizing dye as listed in tabel IV

5 g

5 g

45 ml

45 ml

0.025 g.

15

The recording layers were charged, exposed and developed as described in Example 3.

20 From the obtained prints the relative speed values were calculated based on a comparison of the spectrally sensitized materials with the material without spectral sensitizer to which arbitrarily the speed value of 100 was given.

25 The relative speed values are listed hereinafter.

Table IV

| No. | Structural formula of spectral sensitizing agent | Relative speed value |
|-----|--------------------------------------------------|----------------------|
| 0   | none                                             | 100                  |
| 1   |                                                  | 250                  |
| 2   |                                                  | 300                  |
| 3   |                                                  | 250                  |
| 4   |                                                  | 160                  |
| 5   |                                                  | 1600                 |
| 6   |                                                  | 160                  |

We claim:

1. A recording process comprising producing by exposure to imagewise modulated electromagnetic radiation a pattern of increased conductivity in a photoconductive insulating recording element comprising an organic photoconductive compound corresponding to the following general formula:



wherein:

each of  $Z_1$  and  $Z_2$  (the same or different) represents the necessary atoms to close a benzene nucleus,  
 $Ar$  represents a phenylene group,  
each of  $R_1$  and  $R_2$  (the same or different) represents hydrogen, an alkyl group, a cycloalkyl group, or a benzyl group.

2. A recording material containing a photoconductive insulating recording layer capable of being charged electrostatically in the absence of active electromagnetic radiation and of retaining the applied charge for a period of time sufficiently long to produce thereon a developed electrostatic charge pattern, characterized in that the recording layer stands in electroconductive relationship to a layer or support with lower resistivity and contains an organic photoconductive compound corresponding to the following general formula:



wherein:

each of  $Z_1$  and  $Z_2$  (the same or different) represents the necessary atoms to close a benzene nucleus,  
each of  $R_1$  and  $R_2$  (the same or different) represents hydrogen, an alkyl group, a cycloalkyl group, or a benzyl group, and  
 $Ar$  represents a phenylene group.

3. A recording process according to claim 1, wherein  $R_1$  and  $R_2$  represent a methyl or benzyl group.

4. A recording process according to claim 1, wherein the photoconductive compound corresponds to the following general formula:



15 wherein:

$Z_1$  and  $Z_2$  have the same significance as in claim 1,  
 $A$  represents an alkylene group or an alkylene chain interrupted by a phenylene group, and  
 $Ar$  represents a phenylene group.

20 5. A method as in claim 1 comprising the steps of producing an electrostatic charge pattern by electrostatically charging and information-wise exposing to electromagnetic radiation said recording element producing thereby an information wise increase of the conductivity in the recording element, and developing the resulting latent electrostatic charge pattern with an electrostatically ultractable substance.

25 6. A process according to claim 1, wherein the recording element is a recording layer that has been applied to a conductive layer or support having a resistivity lower than that of the dark-adapted recording element.

30 7. A process according to claim 6, wherein the conductivity layer or support has a resistivity at least  $10^2$  as low as that of the recording element in the dark.

35 8. A recording material according to claim 2, wherein the photoconductive compound corresponds to the following general formula:



40 wherein

45 50  $Z_1$  and  $Z_2$  have the same significance as in claim 2,  
 $A$  represents an alkylene group or an alkylene chain interrupted by a phenylene group, and  
 $Ar$  represents a phenylene group.

\* \* \* \* \*

UNITED STATES PATENT AND TRADEMARK OFFICE  
CERTIFICATE OF CORRECTION

PATENT NO. : 3,912,509

DATED : October 14, 1975

INVENTOR(S) : Wilhelmus Janssens et al

It is certified that error appears in the above-identified patent and that said Letters Patent are hereby corrected as shown below:

In the Claims:

Column 26, line 27 "ultractable" should read

-- attractive --.

Signed and Sealed this  
thirteenth Day of April 1976

[SEAL]

Attest:

RUTH C. MASON

Attesting Officer

C. MARSHALL DANN

Commissioner of Patents and Trademarks